

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## METHOD OF SIZING CARBONATE FILLED PAPER

No Drawing.

Application filed September 5, 1928. Serial No. 304,175.

This invention relates to a method of sizing paper and more particularly to a method of sizing paper filled with carbonate filler.

The principal object of this invention is to provide a method of sizing paper filled with carbonate filler wherein previously mixed sizing is added to the paper mix at the wet end of the paper machine.

Other objects and advantages of this invention will become apparent during the course of the following description.

As is known, when rosin size and alum are added in the beater, mixer, or the like to fibrous material, and carbonate filler is then added, the sizing effect of the rosin size and alum is materially deteriorated, sometimes even to the point of destruction, by the carbonate filler before the paper mix passes on to a web-forming device of a paper machine with the result that the finished paper made from such a mix is incompletely sized, or, in some cases, substantially unsized.

I have discovered that it is possible to avoid this deterioration or destruction of the sizing by mixing rosin size and alum, both preferably in dilute solutions, in a separate container and adding the resulting product, preferably continuously, to the fibrous mix containing carbonate filler at the wet end of the paper machine.

In the preferred practice of my process I mix in a separate container rosin size with an excess of alum. The precipitate may be separated as by filtration from the precipitating bath and used in this condition, or it may be dried and employed in the dried condition after suitable comminution, but these procedures are unnecessary as the soluble by-products of the rosin size-alum reaction do not appear to be detrimental in the process. The precipitate, therefore, together with the accompanying liquid in the separate container is added to the fibrous mix containing carbonate filler preferably continuously at the wet end of the paper machine. However in view of the fact that it is somewhat difficult to disperse flocks of sizing and to distribute them properly in the paper mix to give a substantially uniform sizing effect, I prefer to pass the precipitated sizing prior to its ad-

dition to the fibrous mix through a dispersing or disintegrating machine such as a colloid mill.

In one modification of my process I have found it advantageous to effect the mixing of rosin size and alum in the presence of other material which may be insoluble, such as fibre or clay, or in the presence of material which may be soluble, preferably colloidally soluble, such as starch or glue. In such a modification, the resulting mix is added, as in the previous instance, to the fibrous stock containing carbonate filler at the wet end of the paper machine. When rosin size and alum are mixed in this manner, the sizing material resulting therefrom is produced either in a form which renders it readily dispersible, as when fibre or clay is used, or in a form which is more finely dispersed, as when starch or glue is used. In either event the result is that the mix is thus much more easily incorporated when added to the stock at the wet end of the paper machine.

By adding the sizing mixture to the fibrous mix containing carbonate filler at the wet end of the paper machine, the previously mixed sizing is thus added at a point where there will be a minimum of intimacy and time of contact of the constituents of the mix before the web is formed. This is necessary as I have found that if the sizing mixture be added when the fibrous mix is in relatively concentrated condition, and particularly when the relatively concentrated mix is subjected to agitation as is normal in stock chests, the sizing effect is very quickly deteriorated even to the point of complete destruction. The sizing effect even when the mix is in the diluted condition is gradually deteriorated, but is substantially unaffected within the time limits that the mix is maintained in the dilute state in the usual paper-making procedure. Moreover, although agitation in the dilute state hastens to a certain extent the deterioration of the sizing effect, the speed of deterioration is not nearly so pronounced as in the concentrated condition, and from a practical standpoint I have found that the agitation to which the diluted mix is subjected prior to delivery onto the

web-forming device does not deteriorate the sizing effect to a substantial degree.

An illustrative furnish suitable for use in the practice of my process is as follows:

5 *Materials added in beater*

|                                                               | Pounds |
|---------------------------------------------------------------|--------|
| Fibrous furnish, e. g. sulphite and soda pulps                | 1700   |
| Carbonate filler, e. g. calcium carbonate magnesium hydroxide | 300    |

10 *Materials mixed in separate container and added proportionately and continuously on dilution*

|                              | Pounds |
|------------------------------|--------|
| Size, e. g. rosin size       | 120    |
| Size precipitant, e. g. alum | 180    |

15 Another illustrative furnish is as follows:

*Materials added in the beater*

|                                                               | Pounds |
|---------------------------------------------------------------|--------|
| Fibrous furnish, e. g. sulphite and soda pulps                | 1460   |
| Carbonate filler, e. g. calcium carbonate magnesium hydroxide | 300    |

20 *Materials mixed in separate container and added proportionately and continuously on dilution*

|                                      | Pounds |
|--------------------------------------|--------|
| Fibre, e. g. sulphite and soda pulps | 240    |
| Size, e. g. rosin size               | 120    |
| Size precipitant, e. g. alum         | 180    |

In the above formulæ, the weights of size and carbonate filler refer to the bone dry basis, the weights of all other ingredients being given on the air dry basis.

The herein described method of sizing may be used alone for producing a sized carbonate filled paper or the method may be used in connection with the methods of sizing paper disclosed in my copending applications Serial No. 262,030, filed March 15, 1928; Serial No. 304,167, filed Sept. 5, 1928; Serial No. 304,168, filed Sept. 5, 1928; Serial No. 304,170, filed Sept. 5, 1928; Serial No. 304,172, filed Sept. 5, 1928; Serial No. 304,173, filed Sept. 5, 1928; Serial No. 304,176, filed Sept. 5, 1928; Serial No. 304,177, filed Sept. 5, 1928.

Of course instead of mixing the rosin size and alum in a separate container, streams of these materials may be so placed as to impinge on one another and the resultant stream be directed into the paper mix at the wet end of the paper machine. This procedure offers no special advantage; as a matter of fact, the mixing of the size and alum is apt to be less complete under this condition than when a separate container is used. Therefore I consider this variation the substantial equivalent of mixing the size and alum in a separate container.

In place of alum as a size precipitant I may use with a measure of success an acid such as sulphuric acid ( $H_2SO_4$ ), an acid salt such as sodium bisulfate ( $NaHSO_4$ ), or a salt of a trivalent metal, such as ferric iron or the other salts of aluminum. Of the aluminum salts available I may use the chloride or the like, but I prefer to use ordinary "alum".

65 In place of rosin size I may use satisfac-

torily in the practice of my process other sizes, for example, soaps, such as the oleates, or any other size derived by treatment with an alkaline substance or the like from material originally of acid characteristics or from other material which likewise is of a partially or completely saponifiable nature, such as saponified beeswax.

By the term "carbonate filler" as employed herein, is intended to be included calcium carbonate, of which lime mud from the causticizing process in one form; calcium carbonate magnesium basic carbonate employed in the paper disclosed in my U. S. Patent No. 1,595,416; calcium carbonate magnesium hydroxide disclosed in my U. S. Patent No. 1,415,391; or other substantially water insoluble normal or basic carbonates of alkaline earth metals, (which expression is herein intended to include magnesium), or compounds, double salts, or physically associated mixtures of these with one or more acid soluble materials of a substantially water insoluble nature. The term "carbonate filler" is also intended to include fibrous material and/or other material such as paper coating constituents or the like containing one or more compounds of the character referred to, such as "old papers" or similar papers, "broke", or the like.

By the term "wet end of the paper machine" is intended to be included those instrumentalities employed in paper manufacture by which and/or in which a relatively concentrated paper mix is diluted, and treated, conveyed or fed up to the point of web-formation, such as the mixing box, regulating and proportioning devices, riffles, troughs, screens, head boxes, inlets, and the like, including also instrumentalities used in the white water cycle.

When I use the term "rosin size" it is to be understood that I mean to include any material produced by the action of alkali, generally in aqueous solution, on rosin, or on natural or synthetic resin acid or acids, regardless of the exact composition of the product or the varying composition which different samples may possess.

When I use the word "paper" herein, I use it in the broad sense to include products of manufacture of all types and of all weights and thicknesses, which contain as an essential constituent a considerable amount of prepared fiber and which are capable of being produced on a Fourdrinier, cylinder, or other forming, felting, shaping or molding machine.

While I have described in detail the preferred embodiment of my invention, it is to be understood that the details of procedure, the proportions of ingredients, and the arrangement of steps may be widely varied without departing from the spirit of the invention or the scope of the subjoined claims.

## I claim:

1. The method of sizing paper filled with carbonate filler comprising separately mixing size and size precipitant, and mixing the resulting product with fibrous material and carbonate filler under conditions favoring the minimizing of the time of contact of the constituents of the mix, and thereafter making paper therefrom.
- 10 2. The method of sizing paper filled with carbonate filler comprising separately mixing size and excess of size precipitant, mixing the resulting product with fibrous material and carbonate filler under conditions favoring the minimizing of the time of contact of the constituents of the mix, and thereafter making paper therefrom.
- 15 3. The method of sizing paper filled with carbonate filler comprising separately mixing size and size precipitant, and mixing the resulting product with fibrous material and carbonate filler under conditions favoring the minimizing of the intimacy and time of contact of the constituents of the mix, and thereafter making paper therefrom.
- 20 4. The method of sizing paper filled with carbonate filler comprising separately mixing size and size precipitant, and mixing the resulting product with fibrous material and carbonate filler at the wet end of the paper machine.
- 25 5. The method of sizing paper filled with carbonate filler comprising separately mixing saponified material and precipitant therefor, and mixing the resulting product with fibrous material and carbonate filler at the wet end of the paper machine.
- 30 6. The method of sizing paper filled with carbonate filler comprising separately mixing size and a salt of a trivalent metal, and mixing the resulting product with fibrous material and carbonate filler at the wet end of the paper machine.
- 35 7. The method of sizing paper filled with carbonate filler comprising separately mixing rosin size and size precipitant, and mixing the resulting product with fibrous material and carbonate filler at the wet end of the paper machine.
- 40 8. The method of sizing paper filled with carbonate filler comprising separately mixing size and a salt of aluminum, and mixing the resulting product with fibrous material and carbonate filler at the wet end of the paper machine.
- 45 9. The method of sizing paper filled with carbonate filler comprising separately mixing size and alum, and mixing the resulting product with fibrous material and carbonate filler at the wet end of the paper machine.
- 50 10. The method of sizing paper filled with carbonate filler comprising separately mixing rosin size and alum, and mixing the resulting product with fibrous material and carbonate filler at the wet end of the paper machine.
- 55 11. The method of sizing paper filled with carbonate filler comprising separately mixing rosin size and excess of alum, and mixing the resulting product with fibrous material and carbonate filler at the wet end of the paper machine.
- 60 12. The method of sizing paper filled with carbonate filler comprising separately mixing size and size precipitant, finely dispersing the resulting product, and mixing the finely dispersed product with fibrous material and carbonate filler at the wet end of the paper machine.
- 65 13. The method of sizing paper filled with carbonate filler comprising separately mixing size and alum, finely dispersing the resulting product, and mixing the finely dispersed product with fibrous material and carbonate filler at the wet end of the paper machine.
- 70 14. The method of sizing paper filled with carbonate filler comprising separately mixing rosin size and size precipitant, finely dispersing the resulting product, and mixing the finely dispersed product with fibrous material and carbonate filler at the wet end of the paper machine.
- 75 15. The method of sizing paper filled with carbonate filler comprising separately mixing rosin size and alum, finely dispersing the resulting product, and mixing the finely dispersed product with fibrous material and carbonate filler at the wet end of the paper machine.
- 80 16. The method of sizing paper filled with carbonate filler comprising separately mixing size and size precipitant in the presence of other material, and mixing the resulting product to a fibrous material and carbonate filler at the wet end of the paper machine.
- 85 17. The method of sizing paper filled with carbonate filler comprising separately mixing size and size precipitant in the presence of colloidal material, and mixing the resulting product with fibrous material and carbonate filler at the wet end of the paper machine.
- 90 18. The method of sizing paper filled with carbonate filler comprising separately mixing size and size precipitant in the presence of colloidally soluble material, and mixing the resulting product with fibrous material and carbonate filler at the wet end of the paper machine.
- 95 19. The method of sizing paper filled with carbonate filler comprising separately mixing size and size precipitant in the presence of starch, and mixing the resulting product with fibrous material and carbonate filler at the wet end of the paper machine.
- 100 20. The method of sizing paper filled with carbonate filler comprising separately mixing rosin size and alum in the presence of starch, and mixing the resulting product with fibrous material and carbonate filler at the wet end of the paper machine.

21. In a process of the character described the step of mixing with fibrous material and carbonate filler the insoluble reaction product of size and size precipitant at the wet end of the paper machine.
22. In a process of the character described the step of mixing with fibrous material and carbonate filler the insoluble reaction product of saponified material and a precipitant therefor at the wet end of the paper machine.
23. In a process of the character described the step of mixing with fibrous material and carbonate filler the insoluble reaction product of rosin size and alum at the wet end of the paper machine.

In testimony whereof I affix my signature.  
**HAROLD ROBERT RAFTON.**

21. In a process of the character described the step of mixing with fibrous material and carbonate filler the insoluble reaction product of size and size precipitant at the wet end of the paper machine.

5 22. In a process of the character described the step of mixing with fibrous material and carbonate filler the insoluble reaction product of saponified material and a precipitant therefor at the wet end of the paper machine.

10 23. In a process of the character described the step of mixing with fibrous material and carbonate filler the insoluble reaction product of rosin size and alum at the wet end of the paper machine.

15 In testimony whereof I affix my signature.  
HAROLD ROBERT RAFTON.

20

#### CERTIFICATE OF CORRECTION.

Patent No. 1,803,650.

Granted May 5, 1931, to

HAROLD ROBERT RAFTON.

It is hereby certified that error appears in the printed specification of the above numbered patent requiring correction as follows: Page 2, line 77, for the word "in" read is; page 3, line 103, claim 16, for "to a" read with; and that the said Letters Patent should be read with these corrections therein that the same may conform to the record of the case in the Patent Office.

Signed and sealed this 11th day of August, A. D. 1931.

(Seal)

Wm. A. Kinnan,  
Acting Commissioner of Patents.

55

60

65

**CERTIFICATE OF CORRECTION.**

**Patent No. 1,803,650.**

**Granted May 5, 1931, to**

**HAROLD ROBERT RAFTON.**

**It is hereby certified that error appears in the printed specification of the above numbered patent requiring correction as follows: Page 2, line 77, for the word "in" read is; page 3, line 103, claim 16, for "to a" read with; and that the said Letters Patent should be read with these corrections therein that the same may conform to the record of the case in the Patent Office.**

**Signed and sealed this 11th day of August, A. D. 1931.**

**(Seal)**

**Wm. A. Kinnan,  
Acting Commissioner of Patents.**